

## UNITED STATES PATENT OFFICE

NORMAN BODEN PILLING, OF ELIZABETH, NEW JERSEY, ASSIGNOR TO THE INTERNATIONAL NICKEL COMPANY, INC., OF NEW YORK, N. Y., A CORPORATION OF DELAWARE

## MALLEABLE NICKEL HAVING IMPROVED WELDING QUALITY

No Drawing.

Application filed September 6, 1929. Serial No. 390,856.

This invention relates to malleable nickel and to its alloys.

One of the objects of the invention is to produce, in sheet or wire or other form, improved malleable nickel and nickel-bearing alloys which exhibit a very marked increase in capacity for being successfully and efficiently welded by fusion methods, and where-in the resulting welds show themselves to be stronger, tougher, more ductile and freer from porosity than heretofore.

A further object of the invention is the provision of a novel method of accomplishing the improved product and its alloys.

It is generally known that, in order to have the quality of malleability, nickel must be processed with and have a certain small amount of magnesium. This function of magnesium is considered to be concerned with the trace of sulphur usually present, insuring that this sulphur content occurs as an infusible magnesium sulphide instead of a fusible nickel sulphide. Experience has taught that nickel, suitably processed with magnesium to yield sound ingots and an excellent degree of malleability (such as will permit reduction to thin sheet and wire) may yield welds which are extremely porous, have a very low strength and break apart when slightly stretched or bent. It is thought that this is possibly one result of the more severe conditions of fusion in welding as compared with melting in furnaces, but it will be shown that the deficiency in welding quality is not due to too slight a margin of magnesium content and cannot be rectified by an increase in magnesium content.

It has now been found that when the content of magnesium is held within certain preferred limits, and at the same time a suitable content of silicon is added, the welding difficulties are eliminated and fusion welds of exceptional quality are obtained. These welds are strong, tough, ductile, and practically free from porosity.

In specifying the preferred contents of magnesium and silicon in nickel, it may be said that the most practical results are obtained when there is .03 as a minimum and .30 percent as a maximum of magnesium present, and when the silicon ranges from .02 to .4 percent. If the amount of magnesium or silicon is below these minima, porosity and low strength develop in the weld. If magnesium is present in greater amount

than .30 percent, an oxidized scum may form on the molten surface having sufficient bulk and tenacity, not only to hinder or prevent the union of the fused surfaces during welding, but even produce enfoldments and seams within the original ingot serious enough to make it practically impossible to produce sheet and wire of good quality. In respect to the silicon content, it is found that as much as 4 percent, may be present without seriously affecting the welding quality. The maximum content is usually limited by the hardness and brittleness it develops. For refined malleable nickel the range of silicon content preferred is .02 to .40 percent, and magnesium from .06 to .15 percent. The advantageous proportion is Si .10 percent, and Mg .12 percent. This gives a nickel which not only may be forged and worked to sheet and wire, but which responds excellently to the several methods of fusion welding. Nickel containing silicon and magnesium in the proportion cited above is therefore excellently adapted for all those uses in which the structure or part is fabricated from sheet, plate, tube or wire forms by welding.

It is to be particularly noted that these improved, satisfactory welds, may be completed successfully without the need of filling wires or electrodes of special composition.

In illustrating the value of the presence of both magnesium and silicon for the purposes herein set forth the results of three sets of oxyacetylene welding tests will be shown. In making these tests a filler wire was used which was substantially identical in composition with the plate metal.

The first group of tests were made with nickels which contained magnesium in the amounts shown below but which contained no silicon.

| Test No. | 1  | 2   | 3   | 4   | 5   |
|----------|----|-----|-----|-----|-----|
| % Mg.    | .0 | .05 | .09 | .15 | .17 |

In each instance the weld discharged sparks and extruded metal while freezing, and each weld was found upon sectionalizing to be porous. With this grade of nickel a content of 02% magnesium is sufficient to give malleability, but a content even eight times greater, of magnesium alone, does not impart soundness to the welds.

The second group of tests were made with

nickels which contained silicon in the percentages indicated below, but with no magnesium present:

| 5 Test No..... | 6 | 7    | 8   | 9   |
|----------------|---|------|-----|-----|
| % Si.....      | 0 | .035 | .17 | .70 |

These welds, although extremely fluid when 10 melted showed extrusion of the metal during freezing. The welds were brittle and porous when sectionalized and showed the development of gas holes.

The third group of tests were made with 15 nickels which contained both silicon and magnesium in the percentages indicated below:

| Test No..... | 10  | 11  | 12  | 13  | 14  |
|--------------|-----|-----|-----|-----|-----|
| 20 % Si..... | .08 | .09 | .09 | .08 | .72 |
| % Mg.....    | .04 | .09 | .14 | .19 | .10 |

These welds froze quietly, and were sound, free from gas holes, strong, tough and very 25 ductile.

These characteristics of toughness, strength and ductility may possibly be best illustrated by considering the following results of oxyacetylene welding tests made with 30 nickels, the first two of which have an improper proportioning of magnesium and silicon, while the last has magnesium and silicon in amounts conforming to the present invention:

| 35 Test No.....                         | 15    | 16    | 17     |
|-----------------------------------------|-------|-------|--------|
| % Si.....                               | .20   | .01   | .21    |
| % Mg.....                               | .02   | .06   | .07    |
| Breaking stress in lbs. per sq. in..... | 3,200 | 2,800 | 33,200 |
| Elongation, % in 2"                     | 0.5   | 1.0   | 10.5   |

Nickel containing silicon and magnesium in the advantageous proportions responds equally well to fusion welding by the carbon arc and metallic arc methods as by gas fusion methods.

It is to be understood that the invention is applicable not only to metallic nickel but to 50 nickel alloys which contain a substantial proportion of nickel such as nickel-copper alloys, Monel-metal, nickel-chromium alloys, etc. It is also to be understood that such nickel or its alloys may contain in addition

small amounts of other elements that are commonly present in the commercial metal such as carbon, manganese and cobalt. It will be understood that various changes, additions and modifications may be made, but such changes, additions and modifications are considered as being within the scope of this invention when they fall within the scope of the following claims:

What I claim is:

1. As an article of manufacture, a welding element composed of more than 95% refined nickel, about 0.20% to about 0.8% silicon and more than about 0.12% to about 0.3% magnesium, said magnesium being present in sufficient amount not only to combine with sulphur present to render it harmless but also to be available for functioning actively during fusion welding. 70

2. As an article of manufacture, a welding element composed of more than 95% refined nickel, about 0.20% to about 0.4% silicon and about 0.15% to about 0.3% magnesium, said magnesium being present in sufficient amount not only to combine with sulphur present to render it harmless but also to be available for functioning actively during fusion welding. 80

3. As an article of manufacture, a welding element composed of more than 95% refined nickel, about 0.20% silicon and about 0.15% magnesium, said magnesium being present in sufficient amount not only to combine with sulphur present to render it harmless but also to be available for functioning actively during fusion welding. 90

4. A sound, strong, tough and ductile fusion weld composed of more than 95% refined nickel, about 0.20% to about 0.8% silicon and more than about 0.12% to about 0.3% magnesium. 100

5. A sound, strong, tough and ductile fusion weld composed of more than 95% refined nickel, about 0.20% to about 0.8% silicon and about 0.15% to about 0.3% magnesium. 110

6. A sound, strong, tough and ductile fusion weld composed of more than 95% refined nickel, about 0.20% silicon and about 0.15% magnesium. 115

In testimony whereof, I have hereunto set my hand.

NORMAN B. PILLING.